

## 1

3,372,123

## METHOD FOR MANUFACTURING LITHIUM-NICKEL-MANGANESE FERRITE MAGNETIC MEMORY CORES

Cornelis Jacobus Esveldt, Evert Willem Gorter, and Hans Peter Peloschek, Emmasingel, Eindhoven, Netherlands, assignors to North American Philips Company, Inc., New York, N.Y., a corporation of Delaware  
No Drawing. Continuation of application Ser. No. 280,490, May 3, 1963. This application May 24, 1966, Ser. No. 552,631  
Claims priority, application Netherlands, May 25, 1962, 278,942  
4 Claims. (Cl. 252—62.61)

## ABSTRACT OF THE DISCLOSURE

A method of manufacturing magnetic core elements, useful as storage elements, and having a rectangular hysteresis loop, in which a mixture of lithium, nickel, manganese, and ferric oxides, after calcining, is compacted into annular cores which are heated to between 1200° C. and 1400° C. for not more than ten minutes in a water-free atmosphere.

This application is a continuation of application Ser. No. 280,490, filed May 3, 1963, now abandoned.

This invention relates to a method of manufacturing magnetic cores for use as storage elements and to magnetic cores manufactured by such a method. Such magnetic cores have the property that the shape of the hysteresis loop approaches rectangularity. The storage elements are used, for example, in electronic computers.

When using magnetic cores as storage elements it is desirable to limit the occurrence of eddy currents as far as possible, so that magnetically soft, oxidic materials are used more and more as raw materials for such cores, which materials have, as is well-known, a very low electric conductivity.

The suitability of such magnetic cores as storage elements is determined by their current pulse characteristics, that is to say by their behaviour under current pulse conditions. Very important in this connection is, for example, the occurrence of a marked difference between the "zero-signal" and the "one-signal" (in the computer techniques distinction is also made between the "undisturbed" one-signal,  $\mu V_1$ , and the "disturbed" one-signal,  $\mu V_1$ , but these magnitudes differ slightly in a good storage element). For this purpose, in addition to a sufficient "rectangularity" of the hysteresis loop, it is necessary that for a given time of rise of the control current, the period which elapses between the beginning of the control current pulse and the moment at which the output voltage of the one-signal attains its maximum value is substantially constant. For practical reasons the beginning of the control current pulse is not used but the moment at which the control current reaches a strength of 10% of its maximum value. The term "peak time" ( $T_p$ ) of a magnetic core is then to be understood to mean the time which elapses between the instant at which the control current reaches a strength of 10% of its maximum value and the instant at which the output voltage of the one-signal, which is produced by the relevant control cur-

## 2

rent pulse, has become maximum. This peak time is naturally dependent upon the time of rise ( $\tau_r$ ) of the control current pulse. In the experiments having led to the present invention, this time of rise was invariably 0.15 microsecond.

Variations in the control pulse characteristics of storage elements occurring due to temperature variations have mostly been corrected hitherto by varying the strength of the control current. Also the whole system of storage elements has been placed in a thermostatically-controlled enclosure to avoid interfering variations in temperature. However, such methods are complicated and laborious. Besides they are unusable, if during operation of the system, temperature differences occur between the individual storage elements because one element is switched over during a given period more frequently than another. It is therefore very important to have for disposal storage elements which not only exhibit a sufficiently great rectangular ratio of the hysteresis loop, but of which also the output voltage of the one-signal, as well as the peak time, are not dependent on temperature or to a small extent only within a wide range of temperatures (preferably between -40° C. and +125° C.).

In the experiments which have led to the present invention it has been found that magnetic cores consisting of lithium-manganese-(nickel) ferrites, within a range of compositions to be defined hereinafter and manufactured by a method described hereinafter, have current pulse characteristics which render them highly suitable for use as storage elements.

The present invention relates to a method of manufacturing magnetic cores suitable for use as magnetic storage elements by sintering a mass of oxides of lithium, manganese, iron and possibly nickel, and/or compounds of said metals which change to the oxides when strongly heated, which mass has been molded before into the desired shape and, presintered at a temperature lower than 800° C., and it is characterised in that the relative quantities of the said metals in the mass to be sintered, expressed in mol percent of the oxides  $\text{Li}_2\text{O}$ ,  $\text{MnO}$ ,  $\text{Fe}_2\text{O}_3$  and possibly  $\text{NiO}$ , are:

2.5 to 16.4 mol percent of  $\text{Li}_2\text{O}$   
0.3 to 68 mol percent of  $\text{MnO}$   
32 to 82 mol percent of  $\text{Fe}_2\text{O}_3$   
0 to 14 mol percent of  $\text{NiO}$

and that the sintering process takes place at a temperature from 1,200° C. to 1,400° C. in air or in a mixture of air and oxygen.

When magnetic cores manufactured in accordance with the invention are compared, as to their suitability for use as storage cores, with known magnetic cores consisting of manganese-magnesium-(zinc) ferrites, manganese-copper-(zinc) ferrites or lithium-manganese ferrites the following is found. Magnetic cores manufactured in accordance with the invention, if containing higher contents of manganese, are distinguished, with properties otherwise equivalent to those of the aforementioned known magnetic cores, by a strikingly high value of the output voltage of the one-signal. In the case of lower contents of manganese they have, as special favorable properties a very low temperature coefficient of the output voltage of the one-signal and a very low temperature coefficient

of the peak time, the other properties being equivalent to those of the relevant known magnetic cores.

Optimum results are obtained if the mass sintered by heating to a temperature from 1,200° C. to 1,400° C. is first cooled at a rate of at most 30° C. per minute to a temperature which is from 100° C. to 600° C. lower and then quenched or, if the mass is sintered by heating to a temperature from 1,200° C. to 1,400° C. at a rate of more than 30° C. per minute is cooled to a temperature which is from 100° C. to 600° C. lower, the mass is maintained at this lower temperature for at least 5 minutes and then quenched.

As previously mentioned, magnetic cores having a substantially rectangular hysteresis loop and built up of

lithium-manganese ferrites were already known. However, they were manufactured by heating to a temperature not higher than 1,200° C. Hitherto it was believed that the volatility of the lithium oxide was an obstacle to the use of heating temperature higher than 1,200° C. However, it has been found that such is not the case, provided it is ensured that the sintering process takes place in a gaseous atmosphere which does not, or substantially not, contain water vapor.

An example now follows to explain the invention.

#### Example

Mixtures of lithium carbonate,  $\text{Li}_2\text{CO}_3$ , manganese carbonate,  $\text{MnCO}_3$ , ferri-oxide,  $\text{Fe}_2\text{O}_3$ , and possible nickel

carbonate,  $\text{NiCO}_3$  were ground in ethanol in a ball mill for 4 hours. The ground products were pre-sintered in air, cooled to room temperature and ground in ethanol in a ball mill for 16 hours. The resulting ground products, after an organic binder had been added, were granulated and pressed into rings at a pressure of 1.5 tons/cm.<sup>2</sup>. These rings were sintered in air by heating to a temperature from 1,200° C. to 1,400° C.

The table below shows further details about the chemical composition and the manufacturing conditions of the magnetic cores, as well as a number of measuring results.

All the measurements were carried out at 25° C. The time of rise ( $\tau_r$ ) of the control current pulse, as previously mentioned, was invariably 0.15 microsecond.

| Method of sintering and cooling |                                          |              |                         |                                |                                   | Measuring Results                                                                                                                                                                                                                           |                         |                                          |                                                                  |      |
|---------------------------------|------------------------------------------|--------------|-------------------------|--------------------------------|-----------------------------------|---------------------------------------------------------------------------------------------------------------------------------------------------------------------------------------------------------------------------------------------|-------------------------|------------------------------------------|------------------------------------------------------------------|------|
| Core No.                        | Composition in mol percent of the oxides |              |                         | Presintering temperature (°C.) | Output V of the zero signal (mV.) | Output V of the disturbed one-signal $\tau V_1$ (mV.)                                                                                                                                                                                       | Peak time $T_p$ (msec.) | Percent in the temperature range per °C. | Temperature coefficient of the peak time $T_p$ , percent per °C. |      |
|                                 | $\text{Li}_2\text{O}$                    | $\text{MnO}$ | $\text{Fe}_2\text{O}_3$ |                                |                                   |                                                                                                                                                                                                                                             |                         |                                          |                                                                  |      |
| 1.....                          | 14.2                                     | 4.9          | 74.6                    | 6.3                            | 750                               | Heated to a peak temperature of 1,320° C. Within a period of 60 seconds, maintained at this temperature for 7 minutes, then cooled to 980° C. in less than 3 minutes, maintained at this temperature for 16 hours, at last quenched in air. | 17                      | 76                                       | 0.40                                                             | 0.0  |
| 2.....                          | 16.35                                    | 3.92         | 79.73                   | -----                          | 750                               | Heated to peak temperature of 1,340° C. Within 60 seconds, maintained at this temperature for 5 minutes, cooled in the oven which has been switched off to 1,000° C. and, at last, quenched in air.                                         | 19                      | 78                                       | 0.38                                                             | 0.30 |
| 3.....                          | 8.7                                      | 26.1         | 65.2                    | -----                          | 750                               | Heated to peak temperature of 1,265° C. Within 60 seconds, maintained at this temperature for 5 minutes, cooled in the oven which has been switched off to 1,000° C. and, at last, quenched in air.                                         | 26                      | 164                                      | 0.25                                                             | 0.48 |
| 4.....                          | 5.0                                      | 50.0         | 45.0                    | -----                          | 700                               | Heated to peak temperature of 1,280° C. Within 60 seconds, maintained at this temperature for 5 minutes, cooled in the oven which has been switched off to 1,000° C. and, at last, quenched in air.                                         | 18.5                    | 120                                      | 0.34                                                             | 0.65 |
| 5.....                          | 14.2                                     | 4.9          | 74.6                    | 6.3                            | 650                               | Heated to peak temperature of 1,350° C. Within 45 seconds, maintained at this temperature for 10 minutes, cooled in the oven which has been switched off to 950° C. and, at last, quenched in air.                                          | 5.5                     | 35                                       | 0.34                                                             | 0.1  |
| 6.....                          | 12.4                                     | 7.45         | 73.95                   | 6.2                            | 750                               | Heated to peak temperature of 1,280° C. Within 60 seconds, maintained at this temperature for 5 minutes, then cooled to 1,000° C. in less than 3 minutes, maintained at this temperature for 20 minutes, at last quenched in air.           | 16                      | 96                                       | 0.38                                                             | 0.38 |
| 7.....                          | 12.4                                     | 1.24         | 73.96                   | 12.4                           | 750                               | Heated to peak temperature of 1,340° C. Within 60 seconds, maintained at this temperature for 5 minutes, then cooled to 1,000° C. in less than 3 minutes, maintained at this temperature for 20 minutes, at last quenched in air.           | 20                      | 60                                       | 0.32                                                             | 0.25 |
| 8.....                          | 14.4                                     | 4.5          | 77.9                    | 3.2                            | 750                               | Heated to peak temperature of 1,340° C. Within 60 seconds, maintained at this temperature for 5 minutes, then cooled to 1,000° C. in less than 3 minutes, maintained at this temperature for 60 minutes, at last quenched in air.           | 20                      | 95                                       | 0.34                                                             | 0.27 |
| 9.....                          | 14.4                                     | 4.5          | 77.9                    | 3.2                            | 750                               | Heated to peak temperature of 1,340° C. Within 60 seconds, maintained at this temperature for 5 minutes, then cooled to 1,000° C. in less than 3 minutes, maintained at this temperature for 60 minutes, at last quenched in air.           | 23                      | 76                                       | 0.36                                                             | 0.36 |

Each of the cores Nos. 1 to 4 and 6 to 9 had an external diameter of 1.3 mm., an internal diameter of 0.8 mm., a height of 0.4 mm. These dimensions were 0.8 mm., 0.5 mm. and 0.2 mm. respectively for the core No. 5.

What is claimed is:

1. A method of manufacturing a ferromagnetic ferrite core having a substantially rectangular hysteresis loop and a temperature coefficient of the peak time and undisturbed one signal not greater than 0.65% per °C. in a temperature range of at least +20 to +80° C. comprising the steps of, forming a mixture of about 2.5 to 16.4 mol percent of  $\text{Li}_2\text{O}$ ; 0.3 to 68 mol percent of  $\text{MnO}$ ; 32 to 82 mol percent of  $\text{Fe}_2\text{O}_3$  and up to 14 mol percent of  $\text{NiO}$ , presintering said mixture at a temperature not greater than about 750° C., finely-dividing the presintered mixture, compacting the finely-divided presintered mixture into an annular body and sintering said body at a temperature of about 1200° C. to 1400° C. for not more than 10 minutes in an atmosphere containing at least as much oxygen as air and substantially free of water-vapor.

2. A method of manufacturing a ferromagnetic ferrite core as defined in claim 1, in which the quantity of  $\text{NiO}$  in the mixture is at least 3.2 mol percent.

3. A method as claimed in claim 2, in which the body after heating to a temperature from 1200° C. to 1400° C. is first cooled at a rate of at most 30° C. per minute to a temperature which is from 100° C. to 600° C. lower and then quenched.

4. A method as claimed in claim 2, in which the body

after heating to a temperature from 1200° C. to 1400° C. is cooled at a rate of more than 30° C. per minute to a temperature which is from 100° C. to 600° C. lower, maintained at this lower temperature for at least 5 minutes and then quenched.

#### References Cited

#### UNITED STATES PATENTS

|    |           |         |                |       |          |
|----|-----------|---------|----------------|-------|----------|
| 10 | 2,882,234 | 4/1959  | Gorter et al.  | ----- | 252—62.5 |
|    | 3,034,987 | 5/1962  | Baltzer        | ----- | 252—62.5 |
|    | 3,038,860 | 6/1962  | Vinal et al.   | ----- | 252—62.5 |
|    | 3,039,962 | 6/1962  | Fortin         | ----- | 252—62.5 |
|    | 3,054,752 | 9/1962  | Leaycraft      | ----- | 252—62.5 |
| 15 | 3,065,182 | 11/1962 | Aghajanian     | ----- | 252—62.5 |
|    | 3,093,588 | 6/1963  | Brown          | ----- | 252—62.5 |
|    | 3,226,328 | 12/1965 | Esveldt et al. | ----- | 252—62.5 |

#### OTHER REFERENCES

20 Aghajanian: High Curie Temperature Square-Loop Ferrites, IBM Technical Disclosure Bulletin, volume 4, No. 12, May 1962, page 85.

TOBIAS E. LEVOW, *Primary Examiner.*

25 R. D. EDMONDS, *Assistant Examiner.*